

# United States Patent Office

2,893,830

Patented July 7, 1959

1

2,893,830

## FERROMAGNETIC MATERIAL OF THE FORMULA $\text{BaFe}_3\text{O}_5\text{F}$ AND ITS PREPARATION

Lothar Heinrich Brixner, Wilmington, Del., assignor to  
E. I. du Pont de Nemours and Company, Wilmington,  
Del., a corporation of Delaware

No Drawing. Application July 19, 1957  
Serial No. 672,883

5 Claims. (Cl. 23—50)

This invention relates to a new ferromagnetic composition represented by the formula  $\text{BaFe}_3\text{O}_5\text{F}$ .

Ferromagnetic materials might broadly be classified into two groups: those with low coercivities, and those with high coercivities. Materials of the former type are useful in transformers, magnetic amplifiers, memory cores, and microwave devices, and include such well-known substances as the Permalloys, silicon irons, and certain ferrites—the ferrites being materials having the general formula  $\text{MO}\cdot\text{Fe}_2\text{O}_3$  where M is a divalent metal. The ferromagnetic materials with high coercivities include the permanent magnetic materials, such as  $\text{BaO}\cdot 6\text{Fe}_2\text{O}_3$ , and manganese bismuthide (MnBi). It follows, obviously, that ferromagnetic materials of high coercivity provide better permanent magnet characteristics than those with low coercivity. The ferromagnetic material described in this invention possesses an exceptionally high intrinsic coercive force, and it is represented by the chemical formula  $\text{BaFe}_3\text{O}_5\text{F}$ . It has a crystalline structure, but this structure is unlike that of such known ferromagnetic materials as the ferrites and  $\text{BaO}\cdot 6\text{Fe}_2\text{O}_3$ , which is of the magneto plumbite type. X-ray analysis indicates that the composition contains none of the uncombined starting materials, and that it is different from the pattern of  $\text{BaFeO}_2\text{F}$  which might be considered to be an intermediate product in the preparation of my new crystalline material.

The ferromagnetic material of my invention may be prepared by starting with a mixture of  $\text{BaCO}_3$ ,  $\text{BaF}_2$  and  $\text{Fe}_2\text{O}_3$  in a molecular ratio of 1:1:1; i.e., in amounts required to form 2 mols  $\text{BaFeO}_2\text{F}$  with the evolution of 1 mol of  $\text{CO}_2$ . This mixture is heated at a temperature of approximately 1000° C., and then cooled to room temperature and pulverized. The pulverized product is mixed with powdered  $\text{Fe}_2\text{O}_3$  in a stoichiometric quantity based on the formation of  $\text{BaFe}_3\text{O}_5\text{F}$ . This mixture is then fired and cooled. The resulting crystalline material is also pulverized, and then compacted into a unitary mass of desired shape by pressing or extruding. This mass is subjected to firing to produce the ferromagnetic material of this invention.

For a clearer understanding of the invention, the following specific example is given. This example is intended to be merely illustrative of the invention and not in limitation thereof. Unless otherwise specified all parts are by weight.

### Example

According to the equation



stoichiometric amounts of reactants were ground together in an agate ball mill to a fineness of —200 mesh. These amounts by weight were 5.454 gms. of  $\text{BaCO}_3$ , 4.8468 gms. of  $\text{BaF}_2$  and 4.4129 gms. of  $\text{Fe}_2\text{O}_3$ . After thorough mixing, the powder was placed in a platinum crucible and heated in air at a temperature of approximately 1000° C. for 4 hours. The crucible was taken from the furnace, allowed to cool to room temperature, and the reaction

2

product was finely pulverized. A portion of this reaction product was tested with hydrochloric acid and was found to be carbonate free. The material was crystalline but not ferromagnetic. X-ray analysis indicated that it was free of uncombined starting materials. Additional  $\text{Fe}_2\text{O}_3$  (1.257 gms.) in a stoichiometric amount according to the following equation:



10 was ground with 1.9226 gms. of the fired material in an agate ball mill to a fineness of —200 mesh. The mixture was then transferred to a platinum crucible and was heated in air to a temperature of approximately 1200° C. and held at this temperature for two hours. The crucible was removed from the furnace, allowed to cool to room temperature, and the contents pulverized to a —200 mesh by grinding in the agate ball mill. The ground material was shaped into a pellet  $\frac{1}{2}$  inch in diameter at a pressure of 190,000 p.s.i. This pellet was subjected to an additional firing at approximately 1200° C. for one hour. The material thus produced was a dark brown-black compact pellet which was useful as a magnet. When examined by X-ray analysis, there was no indication of the uncombined components which were present prior to the last firing. The magnetic properties as determined with a pressed cylindrical specimen of density 3.96 gm./cc. were as follows:

30  $B_s$ , saturation magnetization ( $4\pi i_s$ ) . 970 gauss.  
 $\sigma_s$ , magnetic moment/gram . . . . . 19.5 ergs/gauss.  
 $B_r$ , remanent magnetization . . . . . 750 gauss.  
 $B_{\max}$ , maximum induction . . . . . 8366 gauss.  
 $BH_{\max}$ , maximum energy product . . . . . 135,790 gauss oersted.

35  $\rho$ , resistivity . . . . .  $10^8 \Omega \text{ cm.}$   
 $iH_c$ , intrinsic coercivity . . . . . 3700 oersteds.

40 The above values of the magnetic properties were obtained with a Sanford-Bennett high field permeameter from the Rubicon Company. A cylindrical sample ( $\frac{1}{2}$  " diameter and about  $1\frac{1}{4}$  " long) was butted between the pole pieces of the permeameter and subjected to the standard operating procedure for obtaining the demagnetizing curve.

45 Alternatively, other decomposable compounds like  $\text{Fe}(\text{NO}_3)_3$  and  $\text{Ba}(\text{NO}_3)_2$  might be used as alternative starting compounds. Commercially available products of the highest purity are preferred as starting materials. Although the example specifies firing temperatures of 1000° C. for the first firing and 1200° C. for the subsequent two firings, both of these temperatures may vary as much as  $\pm 100$ ° C. without effecting any substantial change in the results obtained. Similarly, the times of heating which have been given in the example as four hours for the first heating, two hours for the second, and one hour for the third, may vary as much as, say,  $\pm 1$  hour for the first and second heating and  $\pm \frac{1}{2}$  hour for the third firings, the shorter times being used with the higher temperatures.

55 It will be seen from the above data on my novel magnetic crystalline material, particularly the values which were obtained for remanent magnetization and for intrinsic coercivity, that this material is valuable as a permanent magnet and would be useful in the many applications known for such a material. Among these would be rotating mechanical couplings, television focusing yokes, refrigerator and cabinet door latches, motors, and generators.

60 Since it is obvious that many changes and modifications can be made in the above-described details without departing from the spirit and scope of the invention, it is 65 to be understood that the invention is not to be limited

to said details except as set forth in the appended claims.

I claim:

1. As a composition of matter, a ferromagnetic material of the chemical formula  $\text{BaFe}_3\text{O}_5\text{F}$ .

2. As a composition of matter, a ferromagnetic material of the chemical formula  $\text{BaFe}_3\text{O}_5\text{F}$ , with an intrinsic coercivity of about 3700 oersteds, a remanent magnetization of about 750 gauss, a maximum energy product of about 135,790 gauss-oersteds and a specific resistance of about  $10^8$  ohm-cm.

3. A process for producing a ferromagnetic material which comprises heating at a temperature of about 900° C.-1100° C. for about 3-5 hours a powdered mixture comprising (1)  $\text{BaF}_2$ , (2) an inorganic iron compound selected from the group consisting of  $\text{Fe}_2\text{O}_3$  and  $\text{Fe}(\text{NO}_3)_3$ , and (3) an inorganic barium compound selected from the group consisting of  $\text{BaCO}_3$  and  $\text{Ba}(\text{NO}_3)_2$ , said barium and iron compounds being present in a molecular ratio of 1:1:1, cooling the product thus obtained, grinding the product to a powder, and incorporating with said powder, powdered  $\text{Fe}_2\text{O}_3$  in a stoichiometric amount according to the equation:



heating the latter mixture at a temperature of about 1100° C.-1300° C. for about 1 hour-3 hours, cooling the product thus obtained, grinding the product to a powder, compacting the powder into a unitary mass and heating said mass at a temperature of about 1100° C.-1300° C. for about  $\frac{1}{2}$  hour-1½ hours to convert said latter mixture to ferromagnetic material of the formula  $\text{BaFe}_3\text{O}_5\text{F}$  and recovering said  $\text{BaFe}_3\text{O}_5\text{F}$  material.

4. A process for producing a ferromagnetic material which comprises heating at a temperature of about 900° C.-1100° C. for about 3-5 hours a powdered mix-

ture comprising  $\text{BaF}_2$ ,  $\text{Fe}_2\text{O}_3$ , and  $\text{BaCO}_3$ , said barium and iron compounds being present in a molecular ratio of 1:1:1, cooling the product thus obtained, grinding the product to a powder, and incorporating with said powder, powdered  $\text{Fe}_2\text{O}_3$  in a stoichiometric amount according to the equation:



heating the latter mixture at a temperature of about 1100° C.-1300° C. for about 1 hour-3 hours, cooling the product thus obtained, grinding the product to a powder, compacting the powder into a unitary mass and heating said mass at a temperature of about 1100° C.-1300° C. for about  $\frac{1}{2}$  hour-1½ hours to convert said latter mixture to ferromagnetic material of the formula  $\text{BaFe}_3\text{O}_5\text{F}$  and recovering said  $\text{BaFe}_3\text{O}_5\text{F}$  material.

5. A process for producing a ferromagnetic material which comprises heating at a temperature of about 1000° C. for about 4 hours a powdered mixture comprising  $\text{BaF}_2$ ,  $\text{Fe}_2\text{O}_3$ , and  $\text{BaCO}_3$ , said barium and iron compounds being present in a molecular ratio of 1:1:1, cooling the product thus obtained, grinding the product to a powder, and incorporating with said powder, powdered  $\text{Fe}_2\text{O}_3$  in a stoichiometric amount according to the equation:



heating the latter mixture at a temperature of about 1200° C. for about two hours, cooling the product thus obtained, grinding the product to a powder, compacting the powder into a unitary mass and heating said mass at a temperature of about 1200° C. for about 1 hour to convert said latter mixture to ferromagnetic material of the formula  $\text{BaFe}_3\text{O}_5\text{F}$  and recovering said  $\text{BaFe}_3\text{O}_5\text{F}$  material.

No references cited.